

2,978,293

**METHOD FOR PROTECTING METAL PARTS BY  
MEANS OF VAPOR-PHASE INHIBITORS OF  
METAL CORROSION**

Ladislav Cerveny, 47 Pristavni, Prague, Czechoslovakia

No Drawing. Filed Nov. 29, 1956, Ser. No. 624,956

Claims priority, application Czechoslovakia Dec. 15, 1955

6 Claims. (Cl. 21—2.5)

The present invention relates to a method for protecting metal parts against corrosion by means of vapour-phase inhibitors, and in particular by means of vapour-phase inhibitors which are organic derivates of chromic acid, passivate all metals and protect them in this way against atmospheric corrosion.

Tests of the protective properties of vapour-phase inhibitors for steel, have proved the advantage of their application for protecting steel products against atmospheric corrosion during long storage or transport overseas. The vapor phase inhibitors, when compared with other temporary preserving agents are distinguished by higher efficiency and substantially simpler application, which is important from the point of view of economy.

A disadvantage of the hitherto known vapour-phase inhibitors is their limitation to specific metals, such as steel, nickel and chromium, which are passivated in a nitrite medium. Other metals such as copper or brass are not protected by nitrite type inhibitors, which even enhance the corrosion of zinc, cadmium and magnesium.

Vapour-phase inhibitors suitable for the protection of all metals were not known heretofore.

The method of the invention provides vapour-phase inhibitors fulfilling all the above requirements.

The inhibitors employed are organic derivates of chromic acid in which a chromium anion is combined with a suitable organic component to form a compound whose vapor pressure is sufficient even at the usual temperature and pressure. The vapours of these organic chromates are soluble in water and produce at the sur-

face of metal articles a medium having protective properties.

Organic derivates of chromic acid with a vapour pressure above  $10^{-5}$  mm. Hg/20° C. are particularly suitable such as the neutral chromic acid ester of tert-butyl alcohol  $[(CH_3)_3C]_2CrO_4$ .

When vapour phase inhibitors are used for the protection of finished products in the course of long storage or transport overseas they offer considerable advantages as compared with temporary preserving agents.

Vapour-phase inhibitors according to the invention compare favorably with the hitherto used inhibitors, such as organic derivates of nitrous acid. Their chief advantage resides in the protection which they afford to all metal articles whether they be made of steel, non-ferrous or light metals, which has not been possible with the hitherto known inhibitors.

I claim:

1. A method of protecting a metal surface against corrosion, comprising contacting the metal surface with an ester of chromic acid in the vapor state.

2. A method as set forth in claim 1, wherein said ester has a vapor pressure of not less than  $10^{-5}$  mm. Hg at 20° C.

3. A method as set forth in claim 1, wherein said ester is a water soluble organic chromate.

4. A method as set forth in claim 1, wherein said ester is a chromic acid ester of a tertiary alcohol.

5. A method as set forth in claim 1, wherein the metal surface is exposed to said ester at ambient temperature and pressure.

6. A method of protecting a metal surface against corrosion, comprising contacting the metal surface with the neutral chromic acid ester of tert-butyl alcohol in the vapor state.

**References Cited in the file of this patent**

**UNITED STATES PATENTS**

|    |           |                |               |
|----|-----------|----------------|---------------|
| 40 | 2,053,024 | Dreyfus        | Sept. 1, 1936 |
|    | 2,294,525 | Waugh          | Sept. 1, 1942 |
|    | 2,582,138 | Lane           | Jan. 8, 1952  |
|    | 2,607,744 | Viles          | Aug. 19, 1952 |
|    | 2,629,649 | Wachter et al. | Feb. 24, 1953 |